

## UNITED STATES PATENT OFFICE

2,648,611

## ADDITION OF UREA TO VISCOSE

George Alvin Richter, Jr., Springfield, Pa., assignor to American Viscose Corporation, Wilmington, Del., a corporation of Delaware

No Drawing. Application November 19, 1947,  
Serial No. 787,023

3 Claims. (Cl. 106—165)

1

This invention relates to fibers and yarns comprising regenerated cellulose characterized by high breaking toughness and low average stiffness, and to the production of such fibers and yarns from viscose.

"Breaking toughness" is defined as the work required to break a given yarn, and has the dimensions gram centimeters per denier centimeter. It is numerically equal to the area under the stress-strain curve obtained from various tensile strength testing machines. "Average stiffness" is a measure of the extensibility of the yarns at a given load and is numerically equal to the ratio of the tensile strength at break, to the elongation at break. The terms "breaking toughness" and "average stiffness" are explained in detail in the paper by Harold De Witt Smith, published in the Proceedings of the American Society for Testing Materials, vol. 44, 1944, pp. 589-90.

In the past, the production of fibers and yarns from viscose having the combined characteristics of high breaking toughness, and low average stiffness, has invariably involved changes in the composition and salt test of the viscose, as well as in the spinning conditions, as compared to the viscoses and spinning conditions normally used for the production of fibers and yarns.

The object of the present invention is to produce fibers and yarns characterized by high breaking toughness and low average stiffness from conventional viscoses having normal sodium hydroxide and cellulose content, of normal salt point (as determined by the standard sodium chloride test), and under normal spinning conditions using aqueous acid coagulating and regenerating baths of normal or conventional composition.

I have found that when urea is present in normal viscose, it exerts a marked effect on the breaking toughness and average stiffness of the fibers and yarns obtained by spinning the viscose into an acid spinning bath.

Fibers and yarns obtained from a normal viscose containing a small amount of urea exhibit increased breaking toughness and lowered average stiffness, as compared to the fibers and yarns obtained from a normal viscose of the same sodium hydroxide and cellulose content and salt point, and under the same spinning conditions, but in the absence of urea admixed with the viscose.

The effective amounts of urea are in the range of from about 1 to 5%, based on the weight of the viscose.

Any normal viscose may be used. Such normal

2

viscose have a sodium hydroxide content of from 6 to 8%, based on the weight of the viscose, cellulose content of from 6 to 8%, based on the weight of the viscose, and salt points in the range of from 3 to 6.

The mixture comprising viscose and from about 1 to 5% of urea by weight may be spun into aqueous acid spinning baths containing from about 8 to 12% sulfuric acid, from about 2 to 5% zinc sulfate, and from about 16 to 20% sodium sulfate, the baths being maintained at normal temperatures of from about 45-55° C.

In all instances, the urea exerts a marked effect upon the breaking toughness and average stiffness of the fibers and yarns obtained. However, in general, the effects of the urea are more noticeable in the case of viscoses having the lower salt points in the range of 3 to 6 stated. The lower the salt point (i. e. the more highly ripened or "aged" the viscose) the greater the increase in the breaking toughness, and the greater the decrease in average stiffness of the fibers and yarns obtained.

The urea may be added at any stage in the course of the viscose production, but preferably the urea is admixed with the viscose immediately after its production and prior to storage thereof for ripening, during storage of the viscose for ripening, or after the viscose has been ripened and immediately prior to spinning the fibers or yarns. The urea does not substantially effect the salt point of the viscose, or the processes which normally take place during ripening thereof.

The following specific examples will serve to illustrate the invention. In carrying out the processes of the examples, the stress-strain curve mentioned by Smith (supra) was obtained by means of the Scott inclined plane tensile strength testing machine which is described in detail in the article by A. Stuart Hunter, entitled "Importance of Uniformity in the Constant Rate of Loading with the Scott Inclined Plane Serigraph," American Silk and Rayon Journal, January 1937.

## Example 1

About 2.5% of urea was added, with stirring, to a viscose containing about 7.8% sodium hydroxide and about 7.5% of cellulose, by weight, and having a salt point of 3. The viscose was then spun into an aqueous bath containing about 9% sulfuric acid, about 4% zinc sulfate, and about 20% sodium sulfate to produce a 40 filament, 150 denier yarn which was given a godet stretch of 75%. On testing, the yarn was found to have a dry breaking toughness of 51.9 g. cm./d. cm. and

## 3

average stiffness of 23.2, wet breaking toughness of 28 g. cm./d. cm. and wet average stiffness of 13.6. This compared with a dry breaking toughness of only 38.8 g. cm./d. cm. and average stiffness of 27.2; wet breaking toughness of 20.9 g. cm./d. cm., and wet average stiffness of 21.5 for a yarn spun from a viscose of the same composition, under the same conditions, but which did not contain urea.

## Example 2

To a viscose containing 7.8% sodium hydroxide and 7.5% cellulose, and having a salt point of 5.9, there was added 1.25% of urea by weight. The viscose was then spun into an aqueous bath containing about 11% sulfuric acid, about 5% zinc sulfate, and about 20% sodium sulfate, to produce a 150 denier, 40 filament yarn, which was given a godet stretch of about 69%. The yarn was after-treated in the usual manner, and dried, after which it was tested for breaking toughness and average stiffness. It was found to have a dry breaking toughness of 51.8 g. cm./d. cm., and average stiffness of 17.0; wet breaking toughness of 37.7 g. cm./d. cm., and wet average stiffness of 9.5. A similar yarn, produced from a viscose of the same salt point and basic composition, but not containing urea, was found to have a dry breaking toughness of only 47.8 g. cm./d. cm. and average stiffness of 18.7, and wet breaking toughness of 32.3 g. cm./d. cm. and average stiffness of 9.9.

## Example 3

About 2.5% of urea was added, with stirring, to a viscose containing about 7.8% sodium hydroxide and about 7.5% cellulose, by weight, and having a salt point of 5.1. The viscose was then spun into an aqueous bath containing about 10.6% sulfuric acid, about 3% zinc sulfate and about 18% sodium sulfate to produce a 40 filament, 150 denier yarn which was given a godet stretch of 53%. On testing, the yarn was found to have a dry breaking toughness of 54.4 g. cm./d. cm., and average stiffness of 11.2; wet breaking toughness of 45.7 g. cm./d. cm., and wet average stiffness of 5.2. This compared with a dry breaking toughness of 48.8 g. cm./d. cm., and average stiffness of 12.6; wet breaking toughness of 34.7 g. cm./d. cm., and wet average stiffness of 5.7 for a yarn spun from the same viscose, under the same conditions, but in the absence of urea.

## Example 4

A yarn was produced from a viscose as described in Example 3, containing 2.5% urea by weight. The spinning conditions were the same as in Example 3 except that the yarn was given a godet stretch of 73%. The yarn had a dry breaking toughness of 51 g. cm./d. cm. and average stiffness of 17.5; wet breaking toughness of 36.1 g. cm./d. cm. and wet average stiffness of 9.5, as compared to a dry breaking toughness of 37.7 g. cm./d. cm. and average stiffness of 20.6, and wet breaking toughness of 24.2 g. cm./d. cm. and wet average stiffness of 11.5, for a yarn produced under the same conditions, from a viscose of the same cellulose and sodium hydroxide content, but not containing urea.

## Example 5

5% of urea, by weight, was added to a viscose containing about 7.7% sodium hydroxide and 7.3% cellulose, and having a salt point of 5.4. The viscose having the urea admixed with it was

## 4

then spun into an aqueous bath containing about 11.1% sulfuric acid, about 4.8% zinc sulfate, and about 19.8% sodium sulfate, to produce a 40 filament, 150 denier yarn which was given a stretch of about 44% between godets. This yarn had a dry breaking toughness of 48.1 g. cm./d. cm. and average stiffness of 10.4; wet breaking toughness of 40.3 g. cm./d. cm. and wet average stiffness of 4.9. A similar yarn, from a viscose of the same sodium hydroxide and cellulose content, and of the same salt point, obtained under the same conditions, but in the absence of urea admixed with the viscose, had a dry breaking toughness of only 45 g. cm./d. cm. and average stiffness of 13.5; wet breaking toughness of 33.6 g. cm./d. cm. and wet average stiffness of 5.9.

## Example 6

5% of urea was added with stirring to a viscose containing about 7.5% sodium hydroxide and about 7.6% cellulose, and having a salt point of 5.4. The viscose was then spun into an aqueous bath containing about 10.9% sulfuric acid, about 4.7% zinc sulfate, and about 20% sodium sulfate, to produce a 40 filament, 150 denier yarn which was given a godet stretch of about 65%. The yarn was then after-treated and dried in the usual way. The dried yarn had a dry breaking toughness of 51.4 g. cm./d. cm. and average stiffness of only 14.9; wet breaking toughness of 32.2 g. cm./d. cm. and wet average stiffness of 4.9. Yarn obtained from a viscose of the same fundamental composition but which did not contain urea was found to have a dry breaking toughness of only 44.4 g. cm./d. cm. and average stiffness as high as 18.8; wet breaking toughness of 25.5 g. cm./d. cm. and wet average stiffness of 9.8.

As is apparent from the foregoing examples, the fibers and yarn spun in accordance with the conventional wet spinning technique from a viscose containing the indicated small amounts of urea are distinguished by increased breaking toughness and decreased average stiffness by virtue of which they are especially well adapted to uses in which they are subjected to severe stresses and strains, such as the flexing to which yarns comprising tire cords are exposed. The fibers and yarns have generally increased tensile strengths ranging from about 2.7 to 3 gms./denier and high elongations of from about 17 to 23%.

As has been indicated, the salt point of the viscose may be from 3 to 6, and the amount of urea present may be from 1 to 5%. Generally speaking, the influence of the urea on the breaking toughness and average stiffness of the yarns and fibers obtained from any given viscose containing normal amounts of cellulose and sodium hydroxide, within the ranges indicated, is most pronounced, the lower the salt point of the viscose within the stated range of 3 to 6. At salt points of from, say, 3 to 4, the effects of the urea on the breaking toughness and average stiffness are more pronounced even when the urea is present in the smaller amounts.

The urea exerts its modifying effects on the properties of the fibers either prior to or during their spinning or at any rate prior to final setting up of the fibers. The fibers, after their withdrawal from the bath and after-processing in accordance with the usual procedures, including final washing, are found to be substantially entirely free of urea.

Since it will be obvious that changes and variations may be made in carrying out the invention,

It will be understood that the invention is not to be limited except as defined in the appended claims.

I claim:

1. A fiber-forming composition consisting of a mixture of viscose containing, by weight, from about 6 to about 8% of sodium hydroxide and from about 6 to about 8% of cellulose, and having a sodium chloride salt test value of from 3 to 6, with from 1 to 5% by weight of urea.

2. As a fiber-forming composition, a mixture of viscose with about 1 to 5% by weight of organic water-soluble material consisting of urea, the urea being the sole organic water-soluble material in the mixture, said composition having normal aging characteristics.

3. As a fiber-forming composition, a mixture of viscose containing about 6 to about 8% of sodium hydroxide by weight and about 6 to about

5

8% by weight of cellulose, with about 1 to 5% by weight of organic water-soluble material consisting of urea, the urea being the sole organic water-soluble material in the mixture, the composition having a sodium chloride salt point of 3 to 6.

GEORGE ALVIN RICHTER, JR.

References Cited in the file of this patent

UNITED STATES PATENTS

| Number    | Name      | Date          |
|-----------|-----------|---------------|
| 2,155,067 | Ubbelohde | Apr. 18, 1939 |
| 2,364,273 | Cox       | Dec. 5, 1944  |

FOREIGN PATENTS

| Number  | Country       | Date           |
|---------|---------------|----------------|
| 332,628 | Great Britain | July 28, 1930  |
| 539,788 | Great Britain | Sept. 24, 1941 |